

## UNITED STATES PATENT OFFICE

2,688,548

## PHOTOGRAPHIC DEVELOPER COMPOSITION

George A. Reynolds, Rochester, N. Y., assignor to  
 Eastman Kodak Company, Rochester, N. Y., a  
 corporation of New Jersey

No Drawing. Application August 3, 1953,  
 Serial No. 372,166

19 Claims. (Cl. 95—88)

1

This invention relates to photographic developers and particularly to methods for accelerating the development rate of photographic developing agents.

A class of silver halide developing agents has come under consideration which in themselves are very weak developing agents for silver halide emulsions even under the most favorable conditions for development.

These developing agents are the iminoascorbic acids and sugar analogs thereof having the following general structure:



wherein R represents a hydroxyl group when n represents a positive integer from 1 to 4 and R represents a hydrogen atom when n represents a positive integer from 2 to 4.

The following compounds are representative of compounds having the above general formula with which my invention is concerned.



imino-l-erythoascorbic acid



imino-l-ascorbic acid



imino-d-glucoascorbic acid

2



imino-6-desoxy-l-ascorbic acid



imino-l-rhamnoascorbic acid



imino-l-fucoascorbic acid



imino-d-glucoheptoascorbic acid

Other compounds contemplated by the invention which have the above general structure are 45 imino-d-ascorbic acid, imino-l-ascorbic acid, imino-isoascorbic acid and other iminoascorbic acid analogs, e. g., imino-sorboascorbic acid, imino- $\omega$ -lactoascorbic acid, imino-maltoascorbic acid, imino-l-araboascorbic acid, imino-d-glucoascorbic acid, imino-d-galactoascorbic acid, imi-

## 3

no-1-guloascorbic acid, and imino-1-alloascorbic acid.

As will be apparent, the above compounds differ principally in the structure of the terminal group  $R-\text{CH}_2-(\text{CHOH})_{n-1}-$  and in some cases the compounds are stereoisomers. The compounds are described in particular by Pigman and Wolfrom, *Advances in Carbohydrate Chemistry*, Academic Press, New York, 1946, pp. 80-82. Accordingly, the above iminoascorbic acid analogs are named to denote the particular sugar from which they can be synthesized. It will be observed that the compounds are non-aromatic and contain the characteristic mononuclear heterocyclic ene-diol group. The compounds are particularly distinguished from aromatic silver halide developing agents such as catechol or pyrogallol which show serious disadvantages such as strong tendency to form colored oxidation products in the development reaction or on contact with the oxygen in the air which products discolor solutions and stain photographic materials.

I have discovered that the developing rate of developer solutions containing the above ene-diol compounds can be markedly accelerated by the addition to the ene-diol silver halide developing compositions of 3-pyrazolidone compounds which themselves are only moderately active developing agents for silver halide. The activity of the resulting developer solution containing both the ene-diol and the pyrazolidone is very much greater than would be expected from summing up the separate activities. An added feature of the ene-diol-pyrazolidone developer compositions resides in the stability of the developing solution. That is, 3-pyrazolidone compounds such as 1-phenyl-3-pyrazolidone, are highly unstable in alkaline developer compositions free of a preservative and tend to darken and lose development activity quickly particularly through aerial oxidation. On the other hand, when development is carried out with the 3-pyrazolidone compounds in the presence of the ene-diol compounds, the latter function as preservatives and the developer is highly resistant to discoloration and loss of activity. Another advantageous characteristic of the ene-diol-pyrazolidone developer compositions is that the developers show little tendency for the formation of silver sludge or for the formation of dichroic stain on silver images. A further advantage is that since the ene-diol compounds are very effective preservatives for the pyrazolidone developing agents and are highly soluble in water, it is possible to prepare concentrated developer compositions more readily than in the case where a less soluble preservative such as sodium sulfite is used. A further characteristic of the ene-diol-pyrazolidone developer compositions of the invention resides in the fact that the compositions behave as strong surface latent image developers as opposed to internal latent image developers, as long as they are free of silver halide solvents such as sodium sulfite. That is, developer compositions containing 3-pyrazolidone compounds have been described in the literature but invariably they have been compounded so as to contain a silver halide solvent such as sodium sulfite as a preservative. In order to convert such a developer composition to a surface latent image developer, I have found it to be necessary to dispense with the silver halide solvent in the developer composition. However, as mentioned, the 3-pyrazolidone developers free of preservative are very unstable. When, according to my

## 4

invention, the ene-diol compounds are incorporated into the 3-pyrazolidone developer compositions, the ene-diol compounds supply the required preservative effect and the surface latent image developer characteristics are maintained. Therefore, the fortuitous choice of 3-pyrazolidone compounds to accelerate the development rate of the ene-diol compounds has resulted in the latter compounds exerting a complementary preservative effect as well as providing a stable 3-pyrazolidone developer system which has surface latent image development characteristics and shows no tendency for physical development. For these reasons the developers of the invention are very useful in color development processes where a black-and-white developer is required.

An additional unexpected feature of the developers containing the 3-pyrazolidone and ascorbic acid compounds resides in the fact that similar developer compositions can be prepared, in which the pyrazolidone is replaced by a conventional developing agent, for example, containing a mixture of N-methyl-p-aminophenol and ascorbic acid, which compositions do not exhibit the mentioned development acceleration effect to any great extent.

The 3-pyrazolidone developer compositions of the invention containing the above ene-diol compounds can be readily converted to internal latent image developer compositions by merely adding a silver halide solvent such as sodium thiosulfate thereto. The resultant internal latent image developer composition, by virtue of the presence of one of the mentioned ene-diol compounds, likewise possesses excellent keeping properties even in the absence of the usual sulfite preservative.

The 3-pyrazolidone silver halide developing agents employed in the developer compositions together with ascorbic acid and its analogs, have the general formula



in which the R groups each represent various substituents such as hydrogen, alkyl or aryl groups, for example,  $\text{R}_1$  can be hydrogen or a group such as alkyl preferably containing from 1 to 4 carbon atoms, or an aryl group of the benzene or naphthalene series substituted or not, and  $\text{R}_2$ ,  $\text{R}_3$ ,  $\text{R}_4$  and  $\text{R}_5$  can be hydrogen atoms, or groups such as alkyl preferably of 1 to 4 carbon atoms or aryl such as phenyl.

The following compounds are representative of 3-pyrazolidone silver halide developing agents which are useful in the developer compositions of the invention:

1. 1-phenyl-3-pyrazolidone
2. 1-p-tolyl-3-pyrazolidone
3. 5-phenyl-3-pyrazolidone
4. 4-methyl-3-pyrazolidone
5. 1-p-chlorophenyl-3-pyrazolidone
6. 1-phenyl-5-phenyl-3-pyrazolidone
7. 1-m-tolyl-3-pyrazolidone
8. 1-phenyl-5-methyl-3-pyrazolidone
9. 1-p-tolyl-5-phenyl-3-pyrazolidone
10. 1-m-tolyl-3-pyrazolidone
11. 1-p-methoxyphenyl-3-pyrazolidone
12. 1-acetamidophenyl-3-pyrazolidone
13. 1 - phenyl - 2 - acetyl - 4,4 - dimethyl - 3 - pyrazolidone

## 5

14. 1-phenyl-4,4-dimethyl-3-pyrazolidone  
 15. 1-m-aminophenyl-4-methyl-4-propyl-3-pyrazolidone  
 16. 1-o-chlorophenyl-4-methyl-4-ethyl-3-pyrazolidone  
 17. 1-m-acetamidophenyl-4,4-diethyl-3-pyrazolidone  
 18. 1-(p- $\beta$ -hydroxyethylphenyl)-4,4-dimethyl-3-pyrazolidone  
 19. 1-p-hydroxyphenyl-4,4-dimethyl-3-pyrazolidone  
 20. 1-p-methoxyphenyl-4,4-diethyl-3-pyrazolidone  
 21. 1-p-tolyl-4,4-dimethyl-3-pyrazolidone  
 22. 1-(7-hydroxy-2-naphthyl)-4-methyl-4-n-propyl-3-pyrazolidone  
 23. 1-p-diphenyl-4,4-dimethyl-3-pyrazolidone  
 24. 1-(p- $\beta$ -hydroxyethylphenyl)-3-pyrazolidone  
 25. 1-o-tolyl-3-pyrazolidone  
 26. 1-o-tolyl-4,4-dimethyl-3-pyrazolidone

The 4,4-dialkyl-3-pyrazolidone compounds 13 to 23 and 26 above are particularly efficacious for use in the developer compositions of my invention inasmuch as they are more active developing agents than are compounds 1 to 12 which contain a single substituent or only hydrogen atoms in the 4-position of the pyrazolidone nucleus. The 4,4-dialkyl-3-pyrazolidone compounds are described and claimed in the Allen et al. U. S. patent application Serial No. 372,148 filed concurrently herewith. The  $\omega$ -hydroxy-alkyl-3-pyrazolidones, for example, compounds

## 6

iminoreductone derivative such as p-aminobenzoic acid reductone, m- and p-aminosalicylic acid reductone and sulfanilic acid reductone are similar in structure to the imino ascorbic acid compounds and their use in developer compositions is disclosed and claimed in the Henn and Reynolds U. S. patent application Serial No. 372,168 filed concurrently herewith.

## Example 1

The striking superadditivity obtained by combining the pyrazolidones and ene-diols, is shown in the following table. It is seen that the individual agents develop only weakly, but that when combined, they develop vigorously, producing images of high density.

These formulas all contained 25 grams of sodium sulfite and 25 grams of monohydrated sodium carbonate per liter, in addition to the indicated developing agents. In each case the pH of the formula was adjusted to 10.0 with acetic acid, to bring all solutions under parallel conditions.

The formulas compare the activity of the ene-diol ascorbic acid alone at an 0.02 molar concentration (3.5 grams per liter), of the pyrazolidone by itself, at 0.0025 molar concentration (0.4 to 0.5 gram per liter), and combinations of the agents in these concentrations. The activity was tested with a fine grain positive film, given a step wedge exposure and developed for a series of times at 68° F. and with high agitation.

| Formula No. | Developing Agents                                | Photographic Activity   |        |               |
|-------------|--------------------------------------------------|-------------------------|--------|---------------|
|             |                                                  | Image Density, 4th Step |        | Gamma, 4 Min. |
|             |                                                  | 2 Min.                  | 8 Min. |               |
| 6551        | Iminoglucoascorbic acid+1-phenyl-3-pyrazolidone. | 1.30                    | 2.10   | 1.2           |
| 6552        | Iminoglucoascorbic acid                          | ( <sup>1</sup> )        | 0.60   | 0.12          |
| 6555        | 1-Phenyl-3-pyrazolidone                          | 0.41                    | 0.78   | 0.62          |

<sup>1</sup> No image.

18 and 24 above, are also especially useful in concentrated formulas, in replenishers and in the presence of high salt concentrations where their increased solubility enables obtaining and holding adequate amounts of the pyrazolidone compound in solution. The compounds are described and claimed in the Allent et al. U. S. patent application Serial No. 372,148 filed concurrently herewith and the Reynolds and Tinker U. S. patent application Serial No. 372,167 filed concurrently.

The ene-diol compounds imino-d-glucoscorbic acid above obtained from d-glucose (J. Chem. Soc. 1934, p. 1194) is representative of a number of ene-diol compounds containing the imino-ascorbic acid group derived from sugars. The compound is of particular value in my invention since its development rate is markedly accelerated by the 3-pyrazolidone silver halide developing agents, particularly 1-phenyl-3-pyrazolidone. The other ene-diol compounds containing the imino group can be prepared by the methods of the reference immediately above from, for example, erythrose, galactose, sorbose, mannose, maltose, and lactose and are likewise useful in the 3-pyrazolidone developer compositions where the latter compounds appreciably accelerate the development rate of the ene-diol compounds. As will be apparent above, the

50 The following developer compositions are particularly suitable as negative developers for color films:

- (1) Without sulfite: Grams/liter  
 Sodium hexametaphosphate 0.5  
 Potassium bromide 1.0  
 Sodium carbonate monohydrate 25.0  
 Potassium iodide 0.002  
 1-phenyl-3-pyrazolidone 1.0  
 Imino-d-glucoscorbic acid 12.5  
 1-phenyl-5-mercapto tetrazole 0.01  
 Water to make 1.0 liter
- (2) With sulfite: Grams/liter  
 Sodium hexametaphosphate 0.5  
 Sodium sulfite 40.0  
 Sodium carbonate monohydrate 25.0  
 Potassium bromide 1.0  
 Potassium iodide 0.002  
 1-phenyl-3-pyrazolidone 1.0  
 Imino-d-glucoscorbic acid 12.5  
 1-phenyl-5-mercapto tetrazole 0.01  
 Water to make 1.0 liter

The developers of this example can be used in any of the well-known processes of color development where a black-and-white developer is required. The developers are especially useful in

mixed grain color processes employing films such as disclosed in Mannes et al. U. S. Patent 2,388,856 or in the Carroll et al. U. S. Patent 2,614,925, October 21, 1952, wherein, for example, is shown a two-layer film, one layer containing blue-sensitive silver halide, the other containing a mixture of green and red-sensitive silver halide grains. When the developers immediately above are used in the color process of the patents as the negative developer for such a film it is observed, particularly with the Formula 1 free of sulfite, that physical development effects are minimized with the result that clean highlights free of stain are obtained and the color developed images have increased saturation because of decreased physical development in the negative developer of the invention.

Results similar to those of the above examples are obtained when developer compositions, containing or free of silver halide solvents, are prepared from mixtures of at least one of the indicated 3-pyrazolidone compounds and at least one of the iminoascorbic acid compounds. The enediol-pyrazolidone developer composition of the above example exhibits internal latent image development characteristics particularly by virtue of the presence of the silver halide solvent. Particularly valuable developer compositions in addition to that exemplified above, are those containing imino-d-glucoascorbic acid and either 1-phenyl-3-pyrazolidone or a 1-tolyl-3-pyrazolidone such as 1-p-tolyl-3-pyrazolidone or 1-p-tolyl-4,4-dimethyl-3-pyrazolidone or a 1-(p- $\beta$ -hydroxyalkylphenyl)-4,4-dialkyl-3-pyrazolidone such as 1-(p- $\beta$ -hydroxyethylphenyl)-4,4-dimethyl-3-pyrazolidone, or a 1-(p- $\beta$ - $\omega$ -hydroxyalkylphenyl)-3-pyrazolidone such as 1-(p- $\beta$ -hydroxyethylphenyl)-3-pyrazolidone.

It will be understood that my invention as specified by the claims hereinafter, includes the mentioned developer compositions in either the liquid form exemplified above, or in the dry powder form as packaged developer formulas suitable for dissolving in water to form a liquid developer. Such dry compositions include the mentioned 3-pyrazolidone compounds, the enediol compound, and alkaline material such as sodium carbonate, caustic alkali or sodium metaborate.

What I claim is:

1. A photographic developer composition comprising an alkaline material, a 3-pyrazolidone silver halide developing agent and a compound having the general structure



wherein R represents a hydroxyl group when n represents a positive integer from 1 to 4 and R represents a hydrogen atom when n represents a positive integer from 2 to 4.

2. A photographic developer composition comprising an aqueous alkaline solution containing a mixture of a 3-pyrazolidone silver halide developing agent and a compound having the general structure



wherein n represents a positive integer from 1 to 4.

3. A photographic developer composition comprising an aqueous alkaline solution containing a mixture of a 3-pyrazolidone silver halide de-

veloping agent and a compound having the structure



4. A photographic developer composition comprising an aqueous alkaline solution containing a mixture of a 3-pyrazolidone silver halide developing agent and a compound having the structure



5. A photographic developer composition comprising an aqueous alkaline solution containing a mixture of a 3-pyrazolidone silver halide developing agent and a compound having the structure



6. A photographic developer composition comprising an aqueous alkaline solution containing a mixture of a 3-pyrazolidone silver halide developing agent and a compound having the structure



7. A photographic developer composition comprising an aqueous alkaline solution containing a mixture of a 3-pyrazolidone silver halide developing agent and imino-d-glucoascorbic acid.

8. The developer composition of claim 2 wherein in the designated 3-pyrazolidone is 1-phenyl-3-pyrazolidone.

9. The developer composition of claim 2 wherein in the designated 3-pyrazolidone is a 4,4-dialkyl-3-pyrazolidone.

10. A photographic developer composition comprising an aqueous alkaline solution containing a mixture of a 1-tolyl-3-pyrazolidone and imino-d-glucoascorbic acid.

11. A photographic developer composition comprising an aqueous alkaline solution containing a mixture of 1-p-tolyl-4,4-dimethyl-3-pyrazolidone and imino-d-glucoascorbic acid.

12. A photographic developer composition comprising an aqueous alkaline solution containing a mixture of 1-phenyl-4,4-dimethyl-3-pyrazolidone and imino-d-glucoascorbic acid.

13. A photographic developer composition comprising an aqueous alkaline solution containing a mixture of 1-(p- $\beta$ -hydroxyethylphenyl)-3-pyrazolidone and imino-d-glucoascorbic acid.

14. A photographic developer composition comprising an aqueous alkaline solution containing a mixture of 1-(p- $\beta$ -hydroxyethylphenyl)-4,4-dimethyl-3-pyrazolidone and imino-d-glucoascorbic acid.

15. A photographic developer composition comprising an aqueous alkaline solution containing a mixture of 1-phenyl-3-pyrazolidone and imino-d-glucoascorbic acid.

16. A photographic developer composition comprising an aqueous alkaline solution containing a mixture of 1-p-tolyl-3-pyrazolidone and imino-d-glucoascorbic acid.

17. A photographic developer composition comprising an aqueous alkaline solution containing

a mixture of a 3-pyrazolidone silver halide developing agent and a compound of the class consisting of imino-L-ascorbic acid, imino-D-ascorbic acid, imino-L-erythroascorbic acid, imino-L-glucouronic acid, imino-D-glucouronic acid, imino-D-galactouronic acid, imino-L-gulouronic acid, imino-L-alloascorbic acid, imino-D-glucouronic acid, imino-L-ramnoascorbic acid, imino-L-fucouronic acid, imino-L-arabouronic acid, imino-sorboascorbic acid, imino-isoascorbic acid, imino-6-desoxy-L-ascorbic acid,

10

imino- $\omega$ -lactoascorbic acid and imino-maltoascorbic acid.

18. The developer composition designated in claim 1 which has been adapted to the development of the internal latent image of exposed silver halide by the addition of a silver halide solvent.

19. The developer composition designated in claim 1 which is free of a silver halide solvent.

No references cited.